

## UNITED STATES PATENT OFFICE

2,138,145

PREPARATION OF ORGANIC DERIVATIVES  
OF CELLULOSE

Camille Dreyfus, New York, N. Y., and George Schneider, Montclair, N. J., assignors to Celanese Corporation of America, a corporation of Delaware

No Drawing. Application November 21, 1935,  
Serial No. 50,872

5 Claims. (Cl. 260—230)

This invention relates to the treatment of organic derivatives of cellulose to remove therefrom compounds which cause solutions of the organic derivatives of cellulose to corrode metal parts with which they come into contact and to remove therefrom compounds which cause haze and cloudy spots in sheets, films and articles made from such organic derivatives of cellulose.

An object of this invention is the economic production of organic derivatives of cellulose which, when dissolved in a liquid solvent, have no corrosive action on metals with which they contact. Another object of the invention is the economic production of a highly transparent organic derivative of cellulose product which is free from haze or cloudy spots. A still further object of this invention is the production of filaments which are uniform in physical characteristics throughout their length. Other objects 20 of the invention will appear from the following detailed description.

Organic derivatives of cellulose, such as cellulose acetate, as ordinarily made contain certain colored constituents or ingredients that tend to impair the usefulness of such derivatives of cellulose in the making of plastics, films, filaments and the like, particularly where transparency and freedom from color are desired. Thus, a thick sheet or block made of a plastic composition containing such derivatives of cellulose has a distinct greenish brown color and is of poor transparency.

Furthermore, such derivatives of cellulose also contain certain constituents or ingredients that tend to corrode metal machine elements and parts of filament-spinning and block pressing devices. For instance, in spinning a solution of cellulose acetate dissolved in a volatile solvent by extruding the same through suitable orifices into an evaporative or precipitating medium, the spinning solutions containing cellulose acetate as normally made tend to corrode the jet holes or orifices. If the corroded material remains in the jet hole, there is produced a filament having a denier below that desired, while if the corroded material is broken away from the jet hole, the jet hole is enlarged and results in a filament having a greater denier than that desired and of undesirable cross-section. It has been the practice heretofore to frequently change the spinning jets and to make periodic examination as to their condition. These operations necessarily interrupt the spinning. Moreover, jet replacements are costly. Furthermore, if improper inspection is made or the jets are not replaced frequently, there is produced a yarn which is not uniform as to denier, cross-section, etc. This non-uniformity of the yarn reflects in the fabric produced from the same, producing a fabric 60 of inferior quality.

Solutions of organic derivatives of cellulose normally have present therein compounds which vary in type and chemical nature and which exhibit different corrosive effects. Thus, one type of corrosive effect is manifested when acetone solutions of cellulose acetate are brought in contact with mercury, resulting in a rapid blackening of the mercury. A second type of corrosive effect is shown by the formation of a brown slimy material which collects about a copper specimen when immersed in the solution containing the organic derivatives of cellulose. This slimy material may be readily dissolved in or dispersed through the solution when it is agitated. A third type of corrosive effect is shown by the production of a green growth about a copper specimen after four or five days' standing in the solution of organic derivatives of cellulose. The fourth type of corrosive effect is shown by the tarnishing of a brightly polished copper specimen, which corrosive effect may be observed after all the first three types have been removed. Products resulting from other types of corrosion may also be present in the organic derivatives of cellulose. However, the above four examples are sufficient to show that the compounds resulting from corrosion have a widely varying chemical nature and produce a wide variation in the type of corrosive effects resulting from contact with metals.

We have found that the compounds produced by corrosive action may be substantially removed from solutions of organic derivatives of cellulose by treating the same with metals. By treating a solution of the organic derivatives of cellulose with metals, the corrosive constituents are either destroyed or are converted into compounds that may be removed by filtering or they may be converted into compounds that tend to reduce such objectionable action to a substantially unappreciable amount.

In accordance with our invention, we prepare derivatives of cellulose of reduced corrosive properties and of reduced color, which derivatives of cellulose are capable of producing products of greater transparency, by treating a flowable solution of the derivatives of cellulose with metals. The treatment may consist in passing the solution through a column containing the metals in a form in which they present a large surface area, whereby the solution contacts with a considerable surface of metal. However, the metals in a finely divided form may be mixed into the solution and then filtered out.

While other derivatives of cellulose, such as cellulose nitrate, may be treated in accordance with this invention, we prefer to treat organic derivatives of cellulose, such as organic esters of cellulose and cellulose ethers. Examples of organic esters of cellulose are cellulose acetate, cel-

lulose formate, cellulose propionate and cellulose butyrate, while examples of cellulose ethers are ethyl cellulose, methyl cellulose and benzyl cellulose.

- 5 The organic derivative of cellulose may be formed by any suitable method. For instance, cellulose acetate may be formed by treating cellulose with acetic anhydride in the presence of a catalyst and a suitable diluent or solvent such 10 as acetic acid. The cellulose acetate thus formed may be subjected to a hydrolysis or ripening treatment to produce the desired solubility characteristics therein. The ripening or hydrolysis may be performed by allowing cellulose acetate, 15 still dissolved in the liquors formed during esterification, to stand for a period of time under suitable temperature conditions. By this process cellulose acetate, which when formed is soluble in chloroform, may be made soluble in acetone. 20 The other esters of cellulose may be formed in a similar manner. For the purpose of describing this invention and in the appended claims, the term "primary solution" refers to a solution of cellulose ester in the solvent produced or added 25 during the esterification of the cellulose. For instance, the primary solution of cellulose acetate, formed in accordance with the above described process, is the acetic acid solution of cellulose acetate containing some sulphuric acid. 30 Although we have found that satisfactory results may be obtained by treating the solutions of the derivatives of cellulose with a metal or metals at any time during their manufacture, we prefer to treat the derivatives of cellulose after they 35 have been precipitated from their primary solution, stabilized and dissolved in a second solution, which second solution may be termed for the purpose of this invention, a "secondary solution". For instance, we may subject the organic derivatives 40 of cellulose to contact with a large surface of metal or metals while the organic derivatives of cellulose are dissolved in their primary solution and after neutralizing a substantial amount of the catalyst employed in their manufacture. 45 The preferred method of carrying out our invention, however, is to first neutralize the catalyst present in the primary solution of the organic derivatives of cellulose, precipitate the organic derivatives of cellulose from the primary solution, stabilize the same by any suitable method 50 and then re-dissolve the organic derivatives of cellulose in any suitable solvent before subjecting the organic derivatives of cellulose to contact with the metal. 55 The solution of organic derivatives of cellulose at the time of treatment with metals may be of any suitable concentration. However, an easily flowable solution is preferred. For cellulose acetate, a suitable working solution may consist of 60 from 5 to 25 parts by weight of cellulose acetate to 75 to 100 parts by weight of acetone. Although any easily flowable solution will give satisfactory results, we prefer to use a solution containing less than 20 per cent of the organic derivatives of cellulose. The organic derivatives of cellulose may be dissolved in a solvent that is to be employed in forming the same into articles and after treating with the metals the solvent 65 may be removed to increase the percentage of organic derivatives of cellulose to the proper working conditions.

The treatment with metals is preferably accomplished by passing a solution of the organic derivatives of cellulose through a column containing the metals in a form presenting a large

surface area. Although any suitable metal, such as zinc, copper, nickel, cobalt, chromium, lead, tin, silver, cadmium, iron, aluminum or other metals, may be employed alone or in series, we prefer to form with two or more metals a voltaic 5 cell or couple. For instance, highly satisfactory results have been produced by intimately mixing copper wool, lead wool and iron wool. The metals may be present in the column in the form of plates, powder, beads, rings, shavings, curls, 10 turnings, etc. To produce the most efficient column metal wool is preferred. The metals, however, may be present in the column in more than one state. For instance, iron wool may be mixed with copper turnings or the iron may be 15 present both as wool and as shavings mixed with copper wool and zinc beads. Any suitable mixture of metals may be employed to form the voltaic cell. The solution may be treated by 20 passing it through a series of columns each containing a single metal or a single column in which there is a series of layers, each layer containing a single metal.

The length of treatment of the solutions of organic derivatives of cellulose with metals depends greatly upon the method of preparing the derivative of cellulose and the types and amounts of corrosive constituents that they contain. For instance, cellulose acetate made as described above and dissolved in acetone may be treated 25 with the metals for from 5 to 60 or more minutes. The length of treatment may be adjusted by regulating the length of the column containing the metals, the rate of flow of material therethrough or by re-circulating the solution through 30 the column several times. Although the treatment with metals at room temperature has been found to be satisfactory, it is preferable to carry out the treatment at a more elevated temperature. For instance, good results may be obtained 40 by passing the solution of organic derivatives of cellulose through the column containing metals at any temperature from 15 to 70 degrees or more but preferably while maintained at a temperature of between 34 to 41° C. 45

The passing of the solution of organic derivatives of cellulose through the column containing metals may be effected by gravity or by flowing the solution through the column under pressure. Whether pressure should be employed depends 50 largely upon the concentration of the derivative of cellulose solution and the length of time the treatment is desired.

Before or after treating the solution of the derivative of cellulose with metal, the solution may 55 be filtered through any convenient type of the many filter presses or continuous rotating filters. As a filtering medium fine cloth, paper, wood pulp or other fibrous material may be used in single or multiple layers. A number of filtrations may be made through the same type of medium or through a different type of medium if desired. Filtrations of the solution containing derivatives of cellulose may be made both before and after treatment with the metals. It is preferable, however, to effect at least one filtration 60 of the solution after treatment with the metals to remove the insoluble compounds produced during the treatment. Two or six or more filtrations may be made through the same or different media. To the solution may be added filter aids such as carbon black, silica gel, fuller's earth or other types of granular or fibrous material which will aid filtration, or absorb color from the 65 solutions. After treatment with the metals, the 70 75

constituents which are not soluble in the solvent may be separated by centrifuging the solution or by filtering and centrifuging the solution.

The derivative of cellulose, when treated by our process, forms plastics, yarns and the like of greater brilliancy, clarity and freedom of color than may be made by an untreated cellulose. It is eminently suitable for making clear plastics that have no pigments or dyes or for the making 5 of light colored plastics. However, the derivative of cellulose produced by our process may be employed for making dark-colored materials.

The derivative of cellulose, when treated by our process, may be formed into sheets and 15 films by casting the same on film-forming wheels and belts formed of metal alloys without corroding the same. Films formed of an untreated derivative of cellulose tend to take on a color or absorb the discolored products of corrosion from 20 the film casting belt or wheel. This property is obviated from the derivative of cellulose produced in accordance with our invention and a solution 25 of such derivatives of cellulose in a volatile solvent therefor may be spun into filaments through spinning jets made of metal alloys with substantially no corrosive action on the spinning jets. Thus, a cellulose derivative produced in accordance with our invention forms more uniform filaments, yarns, straws, etc. than those made of 30 untreated derivatives of cellulose. The spinning into filaments or yarns of an organic derivative of cellulose, treated in accordance with the present invention, is also more economical than the spinning of untreated derivatives of cellulose in 35 that the periods of inspection of the jet orifice may be less frequent and the replacing of jets substantially eliminated.

The derivative of cellulose treated in accordance with our invention may be dissolved with 40 volatile solvents therefor, and may have incorporated therein plasticizers, such as triacetin, diethyl tartrate, dibutyl tartrate, diethyl phthalate, triphenyl phosphate, or other suitable plasticizers by any known processes, to form plastic 45 sheets, blocks, tubes, rods or other articles by any suitable process. Another important application of this invention is in the making of molding powders containing a purified derivative of cellulose in finely divided condition together with 50 plasticizers but containing little or substantially no volatile solvents, which molding powders may be molded under heat and pressure to the desired shape. Films to be employed as a base for photographic or cinematographic films or for other 55 purposes may also be made from this improved derivative of cellulose material. The purified derivative of cellulose may also be used for making lacquers, particularly clear or light colored lacquers. The derivatives of cellulose made in 60 accordance with this invention, being substantially non-corrosive, are particularly suitable for use where solutions of the same in volatile solvents are caused to repeatedly or continuously contact with the same metal surfaces.

65 In order further to illustrate our invention but without being limited thereto, the following specific example is given:

*Example*

70 A 10% by weight solution of cellulose acetate in acetone is passed three times through a four-foot pad of a loosely packed mixture of copper wool, lead wool and iron wool. The pressure on

the solution is adjusted such that the flow of cellulose acetate through the pad requires approximately 20 minutes. The solution is then passed through a filter pad consisting of a six 5 inch layer of wood pulp maintained in position by a layer of cotton cloth on either side. The resulting solution is found to be substantially free of corrosive materials and when formed into a film is free of haze and cloudy spots.

The cellulose acetate solution of the above example may be concentrated, by removing a part 10 of the acetone solvent, to a consistency suitable for forming filaments by the dry method of spinning. When formed into filaments by extruding the same through orifices it produces a substantially uniform filament without affecting by corrosion the diameter of the orifice.

It is to be understood that the foregoing detailed description is given merely by way of illustration and that many variations may be made 20 therein without departing from the spirit of our invention.

Having described our invention, what we desire to secure by Letters Patent is:

1. Process for improving the properties of substitution derivatives of cellulose in which the substituent group is organic, which comprises treating said derivatives of cellulose for at least 5 minutes, while in solution, at a temperature between 34° and 41° C. with a metal in the form 25 of a metal powder, metal wool or similar form presenting a large surface area and thereafter separating such solution from the metal.

2. Process for improving the properties of substitution derivatives of cellulose in which the substituent group is organic, which comprises treating them for at least 5 minutes, while in solution 30 and at a temperature between 34° and 41° C., with metals in the form of metal wool and thereafter separating such solutions from the 40 metals.

3. Process for improving the properties of cellulose acetate, which comprises treating cellulose acetate for at least 20 minutes, while dissolved in more than five times its weight of a liquid 45 solvent and at a temperature between 34° and 41° C., with a plurality of metals in the form of metal powders, metal wool or similar forms presenting a large surface area and thereafter separating such solution from the metals.

4. Process for improving the properties of cellulose acetate, which comprises treating cellulose acetate for at least 5 minutes, while dissolved in more than five times its weight of a liquid solvent and at a temperature between 34° and 41° C., simultaneously with two metals which form a 55 voltaic couple, each of which is in the form of a metal powder, metal wool or similar form presenting a large surface area and thereafter separating the solution from the metals.

5. Process for improving the properties of cellulose acetate which has been precipitated from its primary solution, stabilized and redissolved in more than five times its weight of a liquid solvent, which comprises treating the solution so formed for at least five minutes at a temperature 60 between 34° and 41° C. with a metal in the form of metal powder, metal wool or similar form comprising a large surface area, and thereafter separating the solution from the metal.

70

CAMILLE DREYFUS.  
GEORGE SCHNEIDER.